

## UNITED STATES PATENT OFFICE

ROBERT D. BONNEY, OF GLEN RIDGE, AND WILLIAM B. COLEMAN, OF KEARNY, NEW JERSEY, ASSIGNORS TO CONGOLEUM-NAIRN, INC., A CORPORATION OF NEW YORK

## METHOD OF TESTING

No Drawing.

Application filed January 21, 1930. Serial No. 422,483.

The present invention contemplates a novel method of determining the moisture content of concrete floors as a guide in ascertaining the readiness of the floor for the reception of an installation of linoleum.

It is a well known fact that linoleum or the like can not be successfully installed over a concrete floor which contains more than a certain amount of free moisture. The reason for this is that such moisture when present in excessive amounts forms an alkaline solution with certain constituents of the concrete and such solution acts to disintegrate the linoleum. Furthermore, because of the fact that concrete is formulated in many different ways and is poured and allowed to set or harden under greatly varying conditions, the period required for the moisture content to become reduced below the maximum safety point varies over wide limits. Accordingly, the elapsed period of time after the concrete has been poured is not a safe criterion of the dryness of the floor and it is therefore necessary to determine in each case whether the concrete floor is in suitable condition to receive the linoleum.

The conventional quantitative method heretofore used in determining the suitability of the floor, consisted in ascertaining the percentage of moisture in a sample taken therefrom by the loss in weight occasioned by heating. This method requires the facilities of a laboratory which is frequently unavailable and also the services of a trained analyst. In addition, a period of one to several days elapses between the time when the sample is taken and the receipt of report on the determination of the moisture content. Numerous simple qualitative methods have been proposed and, to some extent, used but none of these offers sufficient accuracy to be accepted as a reliable quantitative method.

It is the object of our invention to overcome all these disadvantages and to provide a quick, simple and reasonably accurate method of determining the readiness of a concrete floor for the reception of an installation of linoleum. More particularly, our invention provides a method which is adapted to be carried out in situ and which

may be completed within 15 to 20 minutes. The method requires neither the equipment of a laboratory nor the services of a trained analyst and may be readily and accurately performed by one unskilled in analytical methods. The above and other advantages will be readily apparent from the following description.

Our novel method is based upon the discovery that calcium carbide or its equivalent when mixed in suitable form and amount with pulverized concrete, reacts exothermically with the free moisture therein, causing a rise in temperature which is directly proportional to the amount of moisture present. Briefly, the method consists in sampling the concrete floor to be tested, pulverizing the sample, admixing in a suitable vessel a predetermined amount of the pulverized concrete with dry powdered calcium carbide, agitating the mix, ascertaining the maximum rise in temperature and converting such temperature rise into terms of percent moisture.

As a specific case, a sample is obtained from the concrete floor to be tested, by drilling. This procedure accomplishes the pulverization of the sample simultaneously with its extraction from the floor. Two cubic centimeters (equivalent to approximately three (3) grams by weight) of the powdered concrete is then measured out by means of a graduated cup and placed in a suitable vessel such as a test tube. An approximately equivalent amount, that is, three (3) grams, of dry powdered calcium carbide is placed in the vessel or test tube above the powdered concrete sample. The sample and calcium carbide are then thoroughly agitated and as the calcium carbide reacts with the moisture of the concrete, heat is generated. The maximum rise in temperature is noted by means of a thermometer, preferably a maximum self-registering thermometer. The extent of the temperature rise serves as a direct measure of the moisture content of the floor. When carrying out the method with a sample of the size described above, the temperature rise will be approximately 12° F. for each percent of moisture present. By di-

viding the maximum rise therefore by 12, the number of percent of moisture is readily determined and the suitability of the floor to receive an installation of linoleum may be ascertained.

5 For convenience, the charge of dry powdered calcium carbide is preferably prepared prior to the test by weighing out the desired amount and sealing the same in a glass tube, or the charge may be otherwise obtained in such form. This facilitates the test and avoids any difficulty which might be encountered in keeping the calcium carbide perfectly dry prior to its use.

10 Certain other substances, capable of reacting exothermically with the free moisture in the concrete, may be used as equivalents for powdered calcium carbide in carrying out our method although because of its availability, cheapness and safety, calcium carbide is to be preferred. Among such other substances may be mentioned calcium phosphide, magnesium nitride, aluminum carbide and sodium peroxide.

15 It will be observed that our invention fills a long felt need in providing a rapid and simple quantitative method of ascertaining in situ the condition of concrete floors. By employing our method, one is able to determine promptly and without elaborate analytical equipment whether a floor is in suitable condition for the reception of an installation of linoleum. It will be apparent that our method is also applicable in determining the moisture content of concrete or plaster walls to ascertain the condition of such surfaces for the reception of paint.

20 Claims:

1. A method of determining the suitability of concrete floors for the reception of an installation of linoleum which comprises the steps of sampling the concrete floor, pulverizing the sample, admixing a determined amount of such sample with an approximately equal amount of dry powdered calcium carbide, agitating the constituents of the mix, and ascertaining the maximum increase in temperature thereof.

2. A method of determining the suitability of concrete floors for the reception of an installation of linoleum which comprises the steps of admixing a determined amount of a pulverized sample of the concrete floor with dry powdered calcium carbide, and ascertaining the maximum increase in temperature of the mix.

3. A method of determining the suitability of concrete floors for the reception of an installation of linoleum which comprises the steps of admixing a determined amount of a pulverized sample of the concrete floor with a substance capable of reacting exothermically with the moisture in said sample and ascertaining the maximum increase in temperature of the mix.

4. A method of determining the moisture content of concrete surfaces or the like which comprises the steps of sampling the surface, pulverizing the sample, admixing a determined amount of the pulverized sample with an approximately equal amount of dry powdered calcium carbide, agitating the constituents of the mix, ascertaining the maximum increase in temperature, and converting the temperature increase into terms of percent moisture.

5. A method of determining the moisture content of concrete surfaces or the like which comprises the steps of sampling the surface, pulverizing the sample, admixing a determined amount of the pulverized sample with a substance capable of reacting exothermically with the moisture in said sample, agitating the constituents of the mix, ascertaining the maximum increase in temperature, and converting said temperature increase into terms of percent moisture.

6. A method of determining the moisture content of concrete surfaces or the like which comprises the steps of admixing a determined amount of a pulverized sample of the concrete surface with dry powdered calcium carbide, and ascertaining the maximum increase in temperature of the mix.

25 In testimony whereof, we affix our signatures.

ROBERT D. BONNEY.  
WILLIAM B. COLEMAN.

100

105

110

115

120

125

130